

225133

## UNITED STATES PATENT OFFICE.

HENRY W. HOLLY, OF BROOKLYN, NEW YORK.

## SLATING COMPOUND FOR ERASABLE TABLETS.

SPECIFICATION forming part of Letters Patent No. 225,133, dated March 2, 1880.

Application filed July 10, 1879.

*To all whom it may concern:*

Be it known that I, HENRY W. HOLLY, of the city of Brooklyn, in Kings county, and State of New York, have invented a certain new and Improved Slating Compound for what are known as "Erasable Tablets," of which the following is a specification.

The white, or nearly white, tablets known as "erasable tablets," and intended for the reception of writing or drawing in black lead-pencil, which is intended to be rubbed out, have been commonly prepared with a coating known as "white slating," which consists of a compound of water-glass and a metallic oxide added thereto to form a "tooth," to enable the tablet to take the pencil freely. Such a compound is entirely non-elastic, and it is found that upon drying the slated surfaces are filled with innumerable fine cracks or fissures, into 20 which the lead of the pencil is rubbed in erasing, thereby in a very short time rendering the tablet unfit for use.

The object of my invention is to furnish a slating compound for such tablets having the required degree of elasticity, which, when spread upon a surface, and dried, forms a smooth, even, and unbroken surface of great durability.

To this end the invention consists in a slat-

ing compound composed of a solution of water-glass, oxide of zinc, and silicate of magnesium. I take about one (1) quart of water-glass of about thirty-nine degrees (39°) Baume and add one (1) quart of water. With the solution thus formed I mix about one (1) pound of pure oxide of zinc powdered and about one (1) pound of powdered silicate of magnesium. When thoroughly mixed a compound of the consistency of paint is formed, which may be readily applied to sheets of stiff paper, board, or other material by means of a brush or otherwise. This compound, when dried, forms a smooth, even, and unbroken surface, from which pencil or other marks may be easily erased, and as said surface contains no cracks or fissures into which the lead of the pencil is rubbed tablets slated with such compound are very durable, and will not become discolored by long use.

What I claim as my invention, and desire to secure by Letters Patent, is—

The slating compound composed of water-glass, oxide of zinc, and silicate of magnesium, substantially as herein specified.

HENRY W. HOLLY.

Witnesses:

HENRY T. BROWN,  
FREDK. HAYNES.